

## 1

3,103,493

## LUBRICATING GREASES

Aleksander Groszek and Geoffrey Hairsine Bell, Sunbury-on-Thames, England, assignors to The British Petroleum Company Limited, London, England, a joint-stock corporation of Great Britain

No Drawing. Filed June 24, 1960, Ser. No. 38,430  
Claims priority, application Great Britain July 2, 1959

18 Claims. (Cl. 252—41)

It is known to prepare lubricating greases by thickening lubricating oils with lithium hydroxy stearate. These greases may, in some cases, be prepared by dissolving pre-formed lithium hydroxy stearate in a lubricating oil at an elevated temperature, rapidly cooling the solution and milling the gel so formed so as to convert it into a grease. In many cases, however, this technique results in the formation of a slurry of coarse granules of soap in the oil. Another method of preparing lithium hydroxy stearate greases is to saponify hydrogenated castor oil in part or all of the oil to be thickened so as to cause the formation of lithium hydroxy stearate in situ. Although somewhat more complicated than the first-mentioned method, this method has the advantage that the glycerol formed during the preparation forms a complex with the soap which imparts good mechanical stability to the grease. Again, however, the formation of a slurry of coarse granules often occurs when this method is used.

We have now found that the formation of lithium hydroxy stearate greases can be facilitated by the use of a particular type of lubricating oil base stock.

According to the invention, there is provided a lubricating grease which has been prepared by thickening to a grease consistency with an alkali metal soap of a hydroxy fatty acid, e.g. an alkali metal soap of a hydroxy stearic acid such as lithium hydroxy stearate, a liquid petroleum lubricating oil base stock consisting of or containing an aromatic fraction which has been separated from a petroleum lubricating oil fraction. Preferably the grease contains 5–15% by weight of the soap.

The liquid lubricating oil base stock may consist of a blend of the aromatic fraction and a petroleum lubricating oil fraction. Particularly suitable blends are those containing at least 10% by weight, e.g. 10–75% by weight, of the aromatic fraction. A suitable petroleum lubricating oil fraction for use in the preparation of the blends is a dewaxed vacuum distillate, particularly a dewaxed vacuum distillate having a viscosity index of at least 40, preferably at least 60, and preferably having a viscosity in the range 45–200 Redwood I seconds at 140° F.

The aromatic fraction may be prepared by selective adsorption of a petroleum lubricating oil fraction on silica gel, activated clay, or other adsorbent material. For example, the lubricating oil fraction may be allowed to flow down a column of silica gel which is thereafter eluted with a solvent which preferentially removes from the adsorbent that part of the oil consisting of saturated hydrocarbons. A suitable solvent for this purpose is a low boiling saturated hydrocarbon e.g. petroleum ether, n-hexane, n-heptane or iso-octane. The aromatic hydrocarbons which remain in the adsorbent together with most of the sulphur-, oxygen- and nitrogen-containing compounds can then be displaced from the adsorbent by a strongly polar, low boiling solvent e.g. acetone, ethyl alcohol, methyl alcohol, isopropyl alcohol, ethyl ether or isopropyl ether. The aromatic fraction recovered after evaporation of the solvent may be used by itself for the preparation of the greases according to the invention, or it may be added to a lubricating oil distillate of the aforementioned type to increase the concentration of aromatics in it.

## 2

Another method that can be used to produce a suitable aromatic fraction is the well-known solvent extraction process. The aromatic extracts obtained by treatment of lubricating oil distillates of the aforementioned type can be used per se as the base stock or they may be added to a lubricating oil distillate to increase its content of aromatic hydrocarbons.

Preferably the lubricating oil base stock is one having an aromatic content of at least 40%, especially at least 50%, by weight as determined by the rapid method of silica gel chromatography described in the Journal of the Institute of Petroleum for July 1958, volume 44, pages 212–215.

Inspection data on several greases is given below in order to illustrate the invention. The greases were prepared from the following base oils:

*Oil A.*—A 160/95 grade lubricating oil (i.e. a lubricating oil having a Redwood I viscosity at 140° F. of 160 secs., and a viscosity index of 95). Oil A contained 29% by weight of aromatics.

*Oil B.*—A 150/75 grade lubricating oil containing 42% by weight of aromatics.

*Oil P.*—An aromatic oil obtained from oil B by adsorption of oil B on a column of silica gel, elution of the saturated hydrocarbons with iso-octane and recovery of the aromatic hydrocarbons by elution with isopropyl alcohol followed by evaporation of the latter. The aromatic fraction obtained in this way amounted to 41.3% by weight of the original oil.

*Oil D.*—A material extracted from a waxy petroleum vacuum distillate by furfural. The undissolved material obtained after this furfural extraction and dewaxing was a lubricating oil of 160/95 grade. Oil D was recovered from solution in the furfural and had a sulphur content of 5.1% by weight and an aromatic content of 87% by weight.

*Oil S.*—A material extracted from a waxy petroleum vacuum distillate by furfural. The undissolved material obtained after the furfural extraction and dewaxing was a lubricating oil of 65/100 grade. Oil S was recovered from solution in the furfural and had a sulphur content of 5.78% by weight and aromatic content of about 85% by weight.

*Oil T.*—A material obtained by hydrofining oil D to reduce its sulphur content. Oil T had a sulphur content of 1.46% by weight and an aromatic content of 80% by weight.

*Oil Q.*—A blend of oil A and oil D containing 75% by weight of oil A and 25% by weight of oil D. Oil Q contained 44% by weight of aromatics.

*Oil R.*—A blend of oil A and oil D containing 50% by weight of oil A and 50% by weight of oil D. Oil R contained 58% by weight of aromatics.

*Oil U.*—A blend of oil A and oil T containing 75% by weight of oil A and 25% by weight of oil T. Oil U contained 42% by weight of aromatics.

*Oil V.*—A blend of oil A and oil T containing 50% by weight of oil A and 50% by weight of oil T. Oil U contained 55% by weight of aromatics.

*Oil W.*—A blend of oil B and oil S containing 75% by weight of oil B and 25% by weight of oil S. Oil W contained 53% by weight of aromatics.

*Oil X.*—A blend of oil B and oil S containing 50% by weight of oil B and 50% by weight of oil S. Oil W contained 63% by weight of aromatics.

The aromatic contents of oils A, B, P, Q and R were determined by the rapid method of silica gel chromatography mentioned above.

## EXAMPLE 1

Two greases according to the invention and two greases for comparison were prepared using pre-formed com-

mercial lithium hydroxy stearate and the base oils A, B and P specified above. Each of the four greases was formed by dissolving the soap in the oil at 225° C., pouring the solution into a cooled tray and milling the gel so formed in a roller mill at 0.005 inch gap. The soap contents and various inspection data on these four greases are given in Table 1, in which greases P1 and P2 are greases according to the invention and greases A1 and B1 are greases prepared for comparison.

Table 1

|                                                   | Grease A1 | Grease B1 | Grease P1 | Grease P2 |
|---------------------------------------------------|-----------|-----------|-----------|-----------|
| Base oil used                                     | Oil A     | Oil B     | Oil P     | Oil P     |
| Content of aromatics in the base oil, percent wt. | 29        | 42        | 100       | 100       |
| Soap concentration, percent wt.                   | 13        | 12        | 11.1      | 9.1       |
| Penetration (IP 50):                              |           |           |           |           |
| Unworked                                          |           | 219       | 115       | 223       |
| 60 strokes                                        |           | 235       | —         | 243       |
| 100,000 strokes                                   |           | 309       | —         | 320       |
| Drop point (IP 31), °C.                           |           | 168       | —         | 196       |
| Bleed Test (DTD 825), percent wt.                 |           | 0.1       | Nil       | 0.6       |

<sup>1</sup> Semi-liquid slurry.

It will be seen that the greases according to the invention (greases P1 and P2) are of good consistency even though smaller soap concentrations than usual were employed. Grease P1 which has a smaller soap concentration than grease B1 has a very much lower penetration. Grease P2 is comparable in penetration and stability with grease B1 although its soap concentration is very much less. Grease P2 also has a satisfactory drop point and gives a satisfactory performance in the bleed test.

#### EXAMPLE 2

Nine greases were prepared to illustrate the properties of greases prepared from hydrogenated castor oil by saponification in situ. Greases prepared by this technique contain glycerol produced from the hydrogenated castor oil. Each sample was prepared by dissolving 13% by weight of hydrogenated castor oil in a lubricating oil base stock at 100° C. Aqueous lithium hydroxide solution was added to saponify the hydrogenated castor oil and the temperature raised to 170° C. to remove the

Table 2

| Grease Number                                     | A2    | Q     | R     | A3    | U     | V     | B2    | W     | X     |
|---------------------------------------------------|-------|-------|-------|-------|-------|-------|-------|-------|-------|
| Base Oil Used                                     | Oil A | Oil Q | Oil R | Oil A | Oil U | Oil V | Oil B | Oil W | Oil X |
| Content of aromatics in the base oil, percent wt. | 29    | 44    | 58    | 29    | 42    | 55    | 42    | 53    | 63    |
| Soap Concentration, percent wt.                   | 13    | 13    | 13    | 13    | 13    | 13    | 13    | 13    | 13    |
| Penetration (IP50):                               |       |       |       |       |       |       |       |       |       |
| Unworked                                          | 253   | 215   | 192   | 256   | 225   | 214   | 239   | 229   | 196   |
| 60 Strokes                                        | 266   | 222   | 199   | 267   | 243   | 232   | 229   | 219   | 206   |
| 100,000 Strokes                                   |       |       |       |       | 303   | 292   | 275   | 293   | 251   |
| Drop Point (IP31), °C.                            | 186   | 178   | 150   | 190   | 193   | 188   | 190   | 189   | 187   |
| Bleed Test (DTD 825), percent wt.                 | 4.3   | 0.2   | Nil   | Nil   | Nil   | Nil   | Nil   | Nil   | Nil   |

final traces of water. The mixture was agitated during saponification and dehydration and stirring was continued until the temperature had fallen to below 100° C. When room temperature had been reached the grease was milled on a roller mill at a 0.005 inch gap and deaerated.

The compositions and various inspection data of the nine greases prepared by the method outlined above are given in Table 2 in which greases Q, R, U, V, W and X are greases according to the invention and greases A2, A3 and B2 are greases prepared for comparison.

It will be seen that greases Q, R, U and V, particularly greases R, have lower penetrations than the corresponding comparative greases A2 and A3. Similarly greases

W and X are of better consistency than the corresponding comparative grease B2.

We claim:

1. A lubricating grease consisting essentially of a petroleum lubricating oil base stock and a thickening agent, in which the thickening agent is an alkali metal soap of a soap-forming hydroxy fatty acid and the petroleum lubricating oil base stock contains at least 40% by weight of an aromatic fraction which has been separated from a petroleum lubricating oil fraction.
- 5 2. A lubricating grease according to claim 1, in which the soap is an alkali metal hydroxy stearate.
3. A lubricating grease according to claim 2, in which the soap is a lithium hydroxy stearate.
- 15 4. A lubricating grease according to claim 1, in which the base stock has been prepared by blending a petroleum lubricating oil fraction and an aromatic fraction which has been separated during the preparation of a petroleum lubricating oil fraction.
- 20 5. A lubricating grease according to claim 4, in which at least one of the petroleum lubricating oil fractions was a dewaxed vacuum distillate.
6. A lubricating grease according to claim 5, in which the dewaxed vacuum distillate had a viscosity index of 25 at least 40.
7. A lubricating grease according to claim 6, in which the dewaxed vacuum distillate had a viscosity index of at least 60.
- 30 8. A lubricating grease according to claim 5, in which the viscosity of the dewaxed vacuum distillate was in the range of 45-200 Redwood I seconds at 140° F.
9. A lubricating grease according to claim 1, in which the base stock contains 40-75% by weight of the aromatic fraction.
- 35 10. A lubricating grease according to claim 1, in which the aromatic fraction was obtained by solvent extraction.
11. A lubricating grease according to claim 1, in which the aromatic fraction was obtained by a chromatographic process.
- 40 12. A lubricating grease according to claim 10, in which the chromatographic process comprised adsorption of the petroleum lubricating oil fraction on an adsorbent material, elution of at least some of the aliphatic materials with a solvent and recovery of the aromatic fraction.
13. A lubricating grease according to claim 12, in which the lubricating oil was adsorbed on an adsorbent selected from the group consisting of silica gel and activated clay.
- 65 14. A lubricating grease according to claim 12, in which the solvent used to elute the aliphatic materials was one selected from the group consisting of petroleum ether, n-hexane and iso-octane.
15. A lubricating grease according to claim 12, in which the aromatic fraction was recovered by elution with a solvent selected from the group consisting of acetone, ethyl alcohol, methyl alcohol, isopropyl alcohol, ethyl ether and isopropyl ether.
- 70 16. A lubricating grease according to claim 1, in which

the aromatic content of the lubricating oil base stock is at least 50% by weight.

17. A lubricating grease according to claim 1, in which the soap was prepared by the saponification in situ of hydrogenated castor oil.

18. A lubricating grease according to claim 1, which contains 5-15% by weight of soap.

References Cited in the file of this patent

UNITED STATES PATENTS

2,625,510 Moore ----- Jan. 13, 1953

UNITED STATES PATENT OFFICE  
CERTIFICATE OF CORRECTION

September 10, 1963

Patent No. 3,103,493

Aleksander Groszek et al.

It is hereby certified that error appears in the above numbered patent requiring correction and that the said Letters Patent should read as corrected below.

Column 3, Table 1, under the column heading "Grease B1", line 6 thereof, for "309" read -- 308 --.

Signed and sealed this 7th day of April 1964.

(SEAL)

Attest:

ERNEST W. SWIDER

Attesting Officer

EDWARD J. BRENNER

Commissioner of Patents